

Jan. 18, 1927.

1,614,846

W. D. MOORE

METHOD OF MAKING METAL CASTINGS

Filed May 29, 1925



INVENTOR

WILLIAM D. MOORE

BY

Franklin Meyer

ATTORNEY

## UNITED STATES PATENT OFFICE.

WILLIAM D. MOORE, OF BIRMINGHAM, ALABAMA, ASSIGNOR TO SAND SPUN PATENTS CORPORATION, OF WILMINGTON, DELAWARE, A CORPORATION OF DELAWARE.

## METHOD OF MAKING METAL CASTINGS.

Application filed May 29, 1925. Serial No. 33,704.

This invention is an improvement in methods of making metal castings, and more particularly in methods of making hollow castings, such as cast iron pipe, in 5 refractory molds.

Such castings are made by introducing molten metal into a refractory mold, supported for rotary movement, and preferably supported for tilting movement, and 10 with the mold inclined during the pouring operation. The mold is rotated while the metal is poured, and in the latter instance it is restored to horizontal position either during the pouring or immediately there- 15 after. That is an additional movement, other than rotary, is imparted to the mold, thereby to modify the circumferential direction of flow of the metal to evenly distribute the same upon the interior of the mold. 20 The castings obtained by centrifugal operation with green sand molds, have desirable properties not obtaining in their entirety in either ordinary sand cast metal, or in centrifugal cast products. Such castings, that 25 is castings made centrifugally in green sand molds combine the superior resistance to corrosion and other disintegrating reactions, characteristic of sand cast metal, with the great density, solidity and strength of centrifugally made castings.

The molds used have heretofore been of metal or of a refractory material such as sand, and with refractory material of every character, the molds have heretofore either 35 been baked in the attempt to eliminate from the sand all the moisture possible, or if not baked they have been faced with a protective facing, as for instance cement, in the manner described in Patent No. 1,471,052, filed Oct. 16, 1923.

The baking and the protective facing are designed to serve somewhat similar functions, among others to prevent cutting and washing of the sand by the molten metal as 45 it flows into the mold; the tendency to the formation of scruff and defects of the pocket or honeycomb type; and instability of the sand lining when subjected to high speeds of rotation; all of which are problems to 50 be solved in centrifugal casting.

The object sought by baking is to make the mold "bone-dry" or substantially so, thus

to remove the moisture which is recognized as the cause of blow holes, gas pockets, segregations of various kinds and the like. 55 The operation is relatively expensive, requiring additional labor, fuel, and time, usually from 6 to 12 hours.

The protective facing may be of the character specified in the above mentioned 60 patent, as for instance a natural cement such as pulverized calcined argillaceous limestone. This is a refractory non-combustible material, capable of fusing with the metal of the casting, and it provides a shell like 65 coating white or grayish white in appearance, and to that extent a departure from the accepted type.

For the reasons above mentioned, as well as to reduce the cost of the operation, and 70 to obtain a more desirable color, and a better finish of the product, it is desirable to produce castings centrifugally in green sand molds, and I have discovered that hollow articles, such as pipe, may be cast in un- 75 baked or "wet" sand molds, without the blowing back of gases, such as would cause blisters, boils and the like, there being sufficient ferro-static pressure to drive the gases through the mold wall.

Some character of facing is however de- 80 sirable to provide a suitable finish for the product, and I have discovered that a suitable material for this purpose is the facing of wet blacking ordinarily used for dry sand work. This facing has for its base a finely 85 comminuted or powdered carboniferous material, and it is applied in a water emulsion. When applied a thick suspension of facing material is left on the mold face. 90

This facing of suspended carboniferous matter, while combustible in oxygen is not consumed during the casting operation, be- 95 cause of the lack of oxygen, nor does it fuse with the metal of the casting. It remains unchanged, except for loss of moisture content. If the casting is permitted to cool before removal from the mold, the carbo- naceous matter will form in a layer which separates easily from the casting, leaving 100 the casting face of a desirable natural dark gray color.

If however the casting should be removed from the mold while it is still hot, that is

while the temperature is sufficiently high to ignite the carboniferous facing material in the presence of oxygen, the facing will be consumed, leaving the casting face of a color 5 much lighter than when the facing is removed mechanically after cooling.

In order to protect those parts of the mold which are subjected to the most violent action of the molten metal during the casting 10 operation, from any possible cutting or washing action, the moisture content of the mold surface over zones which are liable to this action may be subjected to the drying action of a flame for a few minutes only, 15 immediately preceding the casting operation.

While I do not wish to restrict the scope of the invention by any unwarranted assumptions, as to the exact action that takes place, I am of the opinion that the mold is 20 first skin dried in effect by fleeting contacts of the inner wall thereof with the molten metal, before the mold wall is completely covered with a layer of molten metal, which might impede the free venting of the vapor 25 first generated, or which might be effected by such vapor to produce blow holes, blisters and the like.

During the pouring of the mold the speed of rotation of the mold is not so rapid that 30 the centrifugal force will hold the molten metal in contact with the mold wall throughout. The metal is carried only to the highest point of the mold, from whence it falls back into the pool of molten metal. Before 35 the centrifugal force is sufficient to hold the metal in contact with the mold wall throughout its travel, the facing and a thin layer of the mold wall immediately behind the facing is dry and at a high temperature.

40 The highest temperature is at the inner face of the mold, and the temperature of the mold wall increases from this face to the outer face. The moisture is subjected to alternate vaporization and condensation as it 45 travels toward the outer wall in a manner to influence its travel in that direction, and it finds its way to the exterior to the mold, and to the vents of the flask without disturbing the inner surface of the mold wall.

50 That portion first vaporized by the molten metal is condensed or absorbed by the wet sand immediately outside of the same, to be again vaporized and recondensed as the temperature rises from within outward. I have 55 been led to these conclusions by the discovery that better results are obtained with the use of an open grained sand, that is a sand relatively free from bending material, other than water.

60 Centrifugally casting in a "wet" sand mold with a wet facing is a radical departure from accepted practice, and so far as I am aware, I am the first in the art to so cast, and while the invention will be described in 65 detail, such description is intended as only

one exemplification of the method, it being understood that various changes may be made without departing from the spirit of the invention as defined in the claims appended hereto.

70 In the drawings is shown a longitudinal section of a mold prepared in accordance with the method, and ready for casting.

In carrying out the improved method, a sand mold is prepared in the usual way, 75 from sand which may be that commonly used, or combined with other materials, in accordance with the ends sought, and when completed the interior of the mold is faced with a water emulsion of non-soluble carboniferous material, such as finely divided anthracite coal, nut coke, or both, modified by other constituents if desired.

80 This facing which is usually of about the consistency of muddy water, is applied to the mold in any usual or desired manner. The facing surfaces the mold, and prevents the molten metal from fusing with the sand. Although combustible in the usual meaning of the word, it is not effected during the 85 casting operation, and when the casting is cooled, it is substantially unchanged, except as to moisture content. It is easily separated from the casting, leaving a natural 90 dark gray colored surface.

95 In some instances, it may be advisable to subject the mold to the action of a flame for a period of approximately five minutes, just prior to the casting operation. This treatment reduces the moisture content of the facing and the sand in zones which are subject to the most severe action of the flowing metal, before the rapid rotation of the mold is initiated. The sand and facing in such zones is almost if not completely dry, 100 and the sand and facing in the zones immediately adjacent the first named zones which are also subject to severe action of the molten metal, but to less degree than the first named zones, have the moisture content materially reduced.

105 Referring to the drawings, in which the moisture content of the sand constituting the mold A in the flask B is indicated, it will be noted that before treatment with the flame, 110 the moisture content of the sand is about 11%. The zones C at the ends of the mold which will be subjected to the most severe action of the molten metal during the casting operation have the moisture content reduced to about 1%, and in adjacent zones D which are subject to a less violent action, the moisture content is reduced to about 5%.

115 So prepared the molds are ready for casting, the molten metal being introduced in any suitable or desired manner. Any preferred form of casting apparatus may be used. An excellent example of the type 120 wherein the pouring operation is done, while the mold is inclined or tilted from the horizon- 125

zontal being shown and described in the above mentioned patent. With this construction, the mold is restored to the horizontal, at the commencement of the pouring 5 operation, or immediately after, thereby to uniformly distribute the molten metal over the mold surface.

When the molten metal is poured into the mold, it strikes the zone C at the spigot end 10 of the pipe, and this zone when the pipe is treated with the gas flame as above specified is almost dry, the moisture content being approximately 1%. The metal then flows over the zone D which is partially dry, and from 15 thence to the bell end of the pipe. The most severe action of the molten metal at the bell end is at the zone C, where the direction of flow changes, and where the speed of the flow is increased to some extent. This zone 20 corresponds to the dry zone at the spigot end, and it will be evident that at the points where the action of the molten metal is most severe it does not come directly into contact with the sand and facing having the highest 25 moisture content.

The moisture content of the sand is slightly increased by the application of the wet facing and the following table shows the approximate moisture content of cross-sections 30 at the different stages and different localities noted:

|                          | Per Cent. |
|--------------------------|-----------|
| 1st original sand        | 10.5      |
| 2nd after blacking       | 11.2      |
| 3rd ready to cast—bead   | 7.8       |
| 4th ready to cast—middle | 11.1      |
| 5th ready to cast—bell   | 8.6       |

The sand used as previously stated is the regular heap sand, with or without the addition of other matter. The wet facing is composed primarily of carbon, which may be obtained by pulverizing nut coke to the fineness of flour and mixing with water and a suitable binder, as for instance clay. After 45 proper soaking and seasoning, the mixture is brought to a fluid state of such nature as will best suit the sand to be coated or faced.

A suitable sand mixture is that specified in the above mentioned patent, which is composed of silica sand, sharp sand, and molding sands mixed in the proportions of about 50% of the first, 35% of the second, and 15% of the third, although other mixtures 55 may be employed.

The liquid facing may be water emulsion of any of the composition facings used in standard foundry practice. All of these facings have a carboniferous material as a base, anthracite coal, plumbago, nut coke or the like, the carboniferous material being finely pulverized, and used by mixing with water, to which may or may not be added a binder, as may be desired, or found suitable in a particular case. The carbon makes up usually 60 80% of the total solids, and the primary 65

purpose of such material is to form a protective coating on sand surfaces, so that the hot metal will not fuse with the sand.

In the usual foundry practice the mold when prepared, and regardless of the method 70 of preparation or the nature of the sand, is submitted to a drying operation in which an attempt is made to bring the mold into a "bone-dry" condition. In the prior patent above mentioned, wet or unbaked sand 75 molds were used with a protective coating which would fuse with the metal, in accordance with the method set forth in application Serial Number 30,609, filed May 15, 1925, becoming a part of the pipe. In the 80 present invention wet or unbaked sand molds are used, faced with a wet carboniferous material which will remain substantially unchanged during the casting operation except for moisture content, and which will not fuse 85 with the metal of the casting.

The distinctive feature of the present invention is the use of a wet, green or unbaked sand mold, faced with a wet facing which will remain substantially unchanged during 90 the casting operation. A facing which will not fuse with the metal, and which will flake easily from the casting, after cooling leaving it of the natural color, and in condition to be treated with a coating of any desired 95 character, such as cement, asphalt, or the like. In the prior patent above mentioned, the facing is of a material refractory and non-combustible, but fusing with and becoming 100 a part of the product.

The mold may be prepared as described in the said patent or in any other suitable manner, with only such modifications in the normal moisture content, as are desired to resist the most violent effects of the molten 105 metal during the inflow thereof into the mold. The invention also contemplates casting in baked refractory molds, with a wet facing, of the character above specified.

I claim:

1. The method of centrifugally casting hollow metal bodies, which comprises charging molten metal into a rotary wet faced green or unbaked sand mold.

2. The method of centrifugally casting hollow metal bodies, which comprises charging molten metal into a rotary wet faced green or unbaked sand mold, having zones of reduced moisture content near its ends.

3. The method of centrifugally casting hollow metal bodies, which comprises charging molten metal into a rotary green or unbaked sand mold provided with a protective facing of a non-fusible solid.

4. The method of centrifugally casting hollow metal bodies, which comprises charging molten metal into a rotary green or unbaked green sand mold, provided with a protective wet facing, of a finely pulverized solid.

5. The method of centrifugally casting hollow metal bodies, which comprises charging molten metal into a rotary green or unbaked sand mold provided with a protective facing of a finely pulverized non-fusible solid, and having zones of reduced moisture content near its ends.
6. The method of centrifugally casting hollow metal bodies, which comprises 10 charging molten metal into a rotary green or unbaked sand mold provided with a protective facing of a finely pulverized non-fusible solid applied in emulsion.
7. The method of centrifugally casting 15 hollow metal bodies, which comprises charging molten metal into a rotary green or unbaked sand mold provided with a wet facing of a finely pulverized non-fusible solid.
8. The method of centrifugally casting 20 hollow metal bodies, which comprises charging molten metal into a rotary green or unbaked sand mold provided with a wet facing of a finely pulverized solid.
9. The method of centrifugally casting 25 hollow metal bodies, which comprises charging molten metal into a rotary green or unbaked sand mold provided with a wet facing of a finely pulverized solid, and having zones of reduced moisture content near its ends.
10. The method of centrifugally casting 30 hollow metal bodies which consists in pouring molten metal into a rotary green sand mold with a non-soluble non-fusible facing, while the mold is in a position inclined to the horizontal, and moving the mold to a substantially horizontal position while the metal is still in a fluid condition.
11. The method of centrifugally casting 35 hollow metal bodies, which consists in pouring molten metal into a rotary inclined green or unbaked sand mold, having a protective facing of non-soluble non-fusible material, and moving the mold to a substantially horizontal position while the metal is still in a fluid condition.
12. The method of centrifugally casting 40 hollow metal bodies, which consists in pouring molten metal into a rotary inclined green or unbaked sand mold provided with a protective facing of non-soluble non-fusible material in emulsion, and with the moisture content thereof lessened over zones subject to the most violent action of the metal, and moving the mold to a substantially horizontal position while the metal is still in a fluid condition.
13. The method of centrifugally casting 45 hollow metal bodies, which consists in pouring molten metal into a rotary inclined green or unbaked sand mold provided with a protective facing of non-fusible material, and having the moisture content thereof lessened over zones near the ends of the mold, and moving the mold to substantially horizontal position while the metal is still in a fluid condition.
14. The method of centrifugally casting 50 hollow metal bodies with bell ends, which consists in inclining, with the bell end downward, a rotary green or unbaked sand mold having a non-soluble non-fusible protective facing, pouring molten metal toward the said end, and moving the mold to a substantially horizontal position while the metal is still in a fluid condition.
15. The method of centrifugally casting 55 hollow metal bodies with bell ends, which consists in inclining, with the bell end downward, a rotary green or unbaked sand mold, provided with a protective non-soluble non-fusible material in emulsion, and leveling the mold while the metal is still in a fluid condition.
16. The method of centrifugally casting 60 hollow metal bodies with bell ends, which consists in inclining, with the bell end downward a rotary green or unbaked sand mold provided with a protective facing of a water emulsion of pulverulent non-soluble material and having the moisture content thereof reduced over zones subject to the most violent action of the molten metal, and rapidly and gently leveling the mold while the metal is still fluid.
17. The method of centrifugally casting 65 hollow metal bodies, which consists in inclining a rotary green sand mold, provided with a protective facing of an emulsion of non-soluble non-fusible material, and skin dried near the ends over zones subject to the most violent action of the molten metal, and quickly leveling the mold while the metal is still fluid.
18. The method of centrifugally casting 70 hollow metal bodies with bell ends, which consists in preparing a green sand mold provided with a protective facing of an emulsion of a non-soluble non-fusible material, skin drying the ends of the mold over zones subject to the most violent action of the molten metal, inclining the mold with the bell end downward, imparting rotation to the mold, and pouring and leveling while the mold is rotating and the metal is still fluid.
19. The method of centrifugally casting 75 hollow metal bodies, which consists in pouring molten metal into an inclined rotary mold of refractory material, provided with a protective facing of an emulsion of a non-soluble non-fusible material, and having a moisture content of about 1 to 5% over zones near the ends of the mold, and of about 11% elsewhere and leveling the mold while the metal is still fluid.
20. The method of centrifugally casting 80 hollow bodies, which consists in pouring molten metal into an inclined rotary green

sand mold faced with an emulsion of a non-fusible solid, and moving the mold bodily in a direction to impart to the metal while it is still in a fluid condition a flow longitudinally of the mold.

21. The method of centrifugally casting hollow metal bodies, which consists in pouring molten metal into an inclined rotary green sand mold faced with a non-fusible solid and quickly leveling the mold while the metal is still in a fluid condition.

22. The method of centrifugally casting hollow metal bodies having bell ends, which consists in pouring molten metal into a rotary green sand mold faced with a non-fusible solid and arranged with the bell end at a lower level than the spigot end, and bodily moving the mold in a direction to impart to the metal while it is still in a fluid condition a flow longitudinally of the mold.

23. The method of centrifugally casting hollow metal bodies which consists in pouring molten metal into an inclined rotary green sand mold faced with a water emulsion of a non-fusible solid having a high content of carbon, and quickly leveling the mold while the metal is still in a fluid condition.

24. The method of centrifugally casting hollow metal bodies, which consists in pouring molten metal into a rotary mold of refractory material, faced with a mixture of a non-fusible solid and water.

25. The method of centrifugally casting hollow metal bodies, which comprises charging molten metal into a wet faced green or unbaked sand mold while it is rotating at a speed insufficient to hold the molten metal on the mold wall, and abruptly increasing the speed of rotation at or near the end of the charging to apply the metal to the wall and retain it thereon.

26. The method of centrifugally casting hollow metal bodies, which comprises charg-

ing molten metal into a wet faced green or unbaked sand mold having zones of reduced moisture content near its ends while it is rotating at a speed insufficient to hold the molten metal on the mold wall, and abruptly increasing the speed of rotation at or near the end of the charging to apply the metal to the wall and retain it thereon.

27. The method of centrifugally casting hollow metal bodies, which comprises charging molten metal into a wet faced green or unbaked sand mold provided with a protective facing of a non-fusible solid, while it is rotating at a speed insufficient to hold the molten metal on the mold wall, and abruptly increasing the speed of rotation at or near the end of the charging to apply the metal to the wall and retain it thereon.

28. The method of centrifugally casting hollow metal bodies, which comprises charging molten metal into a wet faced green or unbaked sand mold provided with a protective facing of a finely pulverized non-fusible solid in emulsion while it is rotating at a speed insufficient to hold the molten metal on the mold wall, and abruptly increasing the speed of rotation at or near the end of the charging to apply the metal to the wall and retain it thereon.

29. The method of centrifugally casting hollow metal bodies, which comprises charging molten metal into an inclined wet faced green sand mold while it is rotating at a speed insufficient to retain the metal on the mold wall, and while the mold is moving into horizontal position, and abruptly increasing the speed when the mold is near in horizontal position to apply the metal to the mold wall.

Signed at Birmingham in the county of Jefferson and State of Alabama this 1st day of April, A. D. 1925.

WILLIAM D. MOORE.